

1

3,010,814

IMPROVED SULFUR-CURED RUBBER-BASE  
SOLID PROPELLANT CONTAINING MAG-  
NESIUM OXIDEDonald E. Carr, Bartlesville, Okla., assignor to Phillips  
Petroleum Company, a corporation of Delaware  
No Drawing. Filed Mar. 19, 1956, Ser. No. 572,195  
14 Claims. (Cl. 52—5)

This invention relates to improved solid propellant compositions and to a method for their preparation. In one of its more specific aspects this invention relates to solid propellants having improved aging characteristics. In another of its more specific aspects this invention relates to a method for preserving high values of tensile strength, elongation and other mechanical properties in a solid propellant composition.

Recently it has been discovered that superior solid propellant materials are obtained comprising a solid oxidant such as ammonium nitrate or ammonium perchlorate, and a rubbery material such as a copolymer of butadiene and a vinylpyridine or other substituted heterocyclic nitrogen base compound, which after incorporation is cured by a quaternization reaction or a vulcanization reaction. Solid propellant mixtures and a process for their production are disclosed and claimed in copending application Serial No. 284,447, filed April 25, 1952, by W. B. Reynolds and J. E. Pritchard.

In the production of such solid propellant compositions, it is desirable that the products have good mechanical properties such as high values of elongation and tensile strength, low modulus characteristics, as well as good burning rates and that these mechanical properties obtain in the cured propellant composition even after a substantial aging period. It is inevitable that these solid propellant compositions will be maintained in storage for varying lengths of time and it is of particular importance that their physical and ballistic characteristics remain unaltered in so far as it is possible.

It is an object of this invention to provide solid propellant compositions which have tensile strength and elongation values which remain high after aging. It is also an object of this invention to provide solid propellant compositions whose burning rate remains substantially constant during an aging or storing period and which show a pronounced decrease in smoke evolution. It is also an object of this invention to provide a method for preparing a solid propellant composition whose mechanical characteristics and burning rate are substantially unaffected by extended periods of storage. It is also an object of this invention to provide a method for preparing a solid propellant composition displaying a decrease in smoke evolution. Other objects and advantages will be apparent to one skilled in the art upon study of this invention.

Broadly the invention comprises a solid propellant composition comprising a solid oxidizer, a binder containing a rubbery copolymer of a conjugated diene with a polymerizable heterocyclic nitrogen base of the pyridine series, compounding agents for curing the binder composition, a burning rate catalyst, and a minor amount of magnesium oxide. The invention also contemplates a method for the preparation of the solid propellant composition. I have discovered that propellant compositions, as above described, possess superior aging characteristics in that tensile strength and elongation values remain high, the burning rate is only slightly altered and in addition such compositions display a pronounced decrease in smoke evolution upon being fired. The amount of magnesium oxide added will usually be in the range of 0.25 to 5 parts by weight per 100 parts by weight of

2

oxidizer-binder mixture. The amount of magnesium oxide can be decreased or increased in order to obtain the desired result. Particularly beneficial results are obtained when zinc oxide is present in the propellant grain.

5 Zinc oxide is ordinarily employed in the binder recipe as a curing agent.

The rubbery polymers employed as binders in the solid propellant compositions of this invention are copolymers of conjugated dienes with polymerizable heterocyclic nitrogen bases of the pyridine series. These copolymers can vary in consistency from very soft rubbers, i.e., materials which are soft at room temperature but will show retraction when relaxed, to those having a Mooney value (ML-4) up to 100. The rubbery copolymers most frequently preferred have Mooney values in the range between 10 and 40. They may be prepared by any polymerization methods known in the art, e.g., mass or emulsion polymerization. One convenient method for preparing these copolymers is by emulsion polymerization at temperatures in the range between 0 and 140° F. Recipes such as the iron pyrophosphate-hydroperoxide, either sugar-free or containing sugar, the sulfoxylate, and the persulfate recipes are among those which are applicable. It is advantageous to polymerize to high conversion as the unreacted vinylpyridine monomer is difficult to remove by stripping.

10 The conjugated dienes employed are those containing from 4 to 6 carbon atoms per molecule and include 1,3-butadiene, isoprene, 2-methyl-1,3-butadiene, 2,3-dimethyl-1,3-butadiene, and the like. Various alkoxy, such as 15 methoxy and ethoxy and cyano derivatives of these conjugated dienes, are also applicable. Thus, other dienes, such as phenylbutadiene, 2,3-dimethyl-1,3-hexadiene, 2-methoxy-3-ethylbutadiene, 2-ethoxy-3-ethyl-1,3-hexadiene, 20 2-cyano-1,3-butadiene, are also applicable in the preparation of the polymeric binders of this invention.

25 Instead of using a single conjugated diene, a mixture of conjugated dienes can be employed. Thus, a mixture of 1,3-butadiene and isoprene can be employed as the conjugated diene portion of the monomer system.

30 The polymerizable heterocyclic nitrogen bases which are applicable for the production of the polymeric materials are those of the pyridine, quinoline, and isoquinoline series which are copolymerizable with a conjugated diene and contain one, and only one,



35 40 45 50 55 60 65 70 75 80 85 90 95 100 substituent wherein R' is either hydrogen or a methyl group. That is, the substituent is either a vinyl or an alpha-methyl-vinyl (isopropenyl) group. Of these, the compounds of the pyridine series are of the greatest interest commercial at present. Various substituted derivatives are also applicable but the total number of carbon atoms in the groups attached to the carbon atoms of the heterocyclic nucleus should not be greater than 15 because the polymerization rate decreases somewhat with increasing size of the alkyl group. Compounds where the alkyl substituents are methyl and/or ethyl are available commercially.

These heterocyclic nitrogen bases have the formula



or



where R is selected from the group consisting of hydrogen, alkyl, vinyl, alpha-methylvinyl, alkoxy, halo, hydroxy, cyano, aryloxy, aryl, and combinations of these groups such as haloalkyl, alkylaryl, hydroxyaryl, and the like; one and only one of the said groups being selected from the group consisting of vinyl and alpha-methylvinyl; and the total number of carbon atoms in the nuclear substituted groups being not greater than 15. Examples of such compounds are

2-vinylpyridine;  
 2-vinyl-5-ethylpyridine;  
 2-methyl-5-vinylpyridine;  
 4-vinylpyridine;  
 2,3,4-trimethyl-5-vinylpyridine;  
 3,4,5,6-tetramethyl-2-vinylpyridine;  
 3-ethyl-5-vinylpyridine;  
 2,6-diethyl-4-vinylpyridine;  
 2-isopropyl-4-nonyl-5-vinylpyridine;  
 2-methyl-5-undecyl-3-vinylpyridine;  
 2,4-dimethyl-5,6-dipentyl-3-vinylpyridine;  
 2-decyl-5-(alpha-methylvinyl)pyridine;  
 2-vinyl-3-methyl-5-ethylpyridine;  
 2-methoxy-4-chloro-6-vinylpyridine;  
 3-vinyl-5-ethoxypyridine;  
 2-vinyl-4,5-dichloropyridine;  
 2-(alpha-methylvinyl)-4-hydroxy-6-cyanopyridine;  
 2-vinyl-4-phenoxy-5-methylpyridine;  
 2-cyano-5-(alpha-methylvinyl)pyridine;  
 3-vinyl-5-phenylpyridine;  
 2-(para-methylphenyl)-3-vinyl-4-methylpyridine;  
 3-vinyl-5-(hydroxyphenyl)-pyridine;  
 2-vinylquinoline;  
 2-vinyl-4-ethylquinoline;  
 3-vinyl-6,7-di-n-propylquinoline;  
 2-methyl-4-nonyl-6-vinylquinoline;  
 4(alpha-methylvinyl)-8-dodecylquinoline;  
 3-vinylisoquinoline;  
 1,6-dimethyl-3-vinylisoquinoline;  
 2-vinyl-4-benzylquinoline;  
 3-vinyl-5-chloroethylquinoline;  
 3-vinyl-5,6-dichloroisoquinoline;  
 2-vinyl-6-ethoxy-7-methylquinoline;  
 3-vinyl-6-hydroxymethylisoquinoline;  
 and the like.

Oxidants which are applicable in the solid propellant compositions of this invention include ammonium, alkali metal, and alkaline earth metal salts of nitric, perchloric, and chloric acids, and mixtures thereof. Ammonium nitrate and ammonium perchlorate are the preferred oxidants for use in the solid rocket fuels of this invention. Specific oxidants include sodium nitrate, potassium perchlorate, lithium chloride, calcium nitrate, barium perchlorate, and strontium chloride. Mixtures of oxidants are also applicable. In the preparation of the solid rocket propellant compositions, the oxidants are powdered to sizes preferably 300 to 10 microns average particle size. The amount of solid oxidant employed is usually a major amount of the total composition and is generally in the range between 50 and 90 percent by weight of the total mixture of oxidant and binder. If desired,

however, less than 50 percent by weight of the oxidant can be used.

Combustion rate catalysts applicable in the invention include ammonium dichromate, iron oxide, potassium dichromate and metal ferrocyanides and ferricyanides. Ferric ferrocyanides, such as Prussian, Berlin, Hamburg, Chinese, Paris, and milori blue, soluble ferric ferrocyanide, such as soluble Berlin or Prussian blue which contains potassium ferric ferrocyanide, and ferric ferrocyanide which has been treated with ammonia, are among the materials which can be used. Ferrous ferricyanide, Turnbull's blue, is also applicable. A particularly effective burning rate catalyst is milori blue which is pigment similar to Prussian blue but having a red tint and is prepared by the oxidation of a paste of potassium ferrocyanide and ferrous sulfate. Other metal compounds such as nickel and copper ferrocyanides can also be employed. The amount of burning rate catalyst used, in the propellant compositions of this invention, are usually in the range of 0 to 15 parts by weight per 100 parts of oxidant and binder mixture with 1 to 4 parts per 100 parts of oxidant and binder mixture being preferred.

The binder contains a rubbery copolymer of the type hereinbefore described and, in addition, there may be present one or more reinforcing agents, plasticizers, wetting agents, and antioxidants. Other ingredients which are employed for sulfur vulcanization include a vulcanization accelerator, a vulcanizing agent such as sulfur, and an accelerator activator, such as zinc oxide.

A general formulation for binder composition prepared by sulfur vulcanization is given below:

|                                              | Parts by weight |
|----------------------------------------------|-----------------|
| Rubber copolymer (as hereinbefore described) | 100             |
| Reinforcing agent                            | 0-50            |
| 35 Plasticizer                               | 0-100           |
| Wetting agent                                | 0-10            |
| Antioxidant                                  | 0-3             |
| Vulcanization accelerator                    | 0-5             |
| 40 Sulfur                                    | 0-2             |
| Zinc oxide                                   | 0-5             |

Reinforcing agents include carbon black, wood flour, lignin, and various reinforcing resins such as styrene-divinylbenzene, methyl acrylate-divinylbenzene, acrylic acid-styrene-divinylbenzene, and methyl acrylate-acrylic acid-divinylbenzene resins.

In general, any rubber plasticizers can be employed in these binder compositions. Materials such as Pentaryl A (amyl biphenyl), Paraflex (saturated polymerized hydrocarbon), Circosol-2XH (petroleum hydrocarbon softener having a specific gravity of 0.940 and a Saybolt Universal viscosity at 100° F. of about 2000 seconds), di(1,4,1-trioxaundecyl)methane designated as TP-90B and available from the Thiokol Corp., and dioctyl phthalate are suitable plasticizers. Materials which provide rubber having good low temperature properties are preferred. It is also frequently preferred that the plasticizers be oxygen-containing materials.

Wetting agents aid in deflocculating or dispersing the oxidizer, Aerosol OT (dioctyl ester of sodium sulfosuccinic acid), lecithin, and Duomeen C diacetate (the diacetate of trimethylene diamine substituted by a coconut oil product) are among the materials which are applicable.

65 Antioxidants include Flexamine (physical mixture containing 25 percent of a complex diarylamine-ketone reaction product and 35 percent of N,N'-diphenyl-p-phenylenediamine), phenyl-beta-naphthylamine, 2,2-methylene-bis(4-methyl-6-tert-butylphenol), and the like. Rubber 70 antioxidants, in general, may be employed or if desired may be omitted.

Examples of vulcanization accelerators include the carbamate type, such as N,N-dimethyl-S-tert-butylsulfonyl dithiocarbamate and Butyl Eight. Butyl Eight is a rubber accelerator of the dithiocarbamate type supplied by

the R. F. Vanderbilt Company and described in "Handbook of Material Trade Names" by Zimmerman and Lavine, 1953 edition, as a brown liquid; specific gravity 1.01; partially soluble in water and gasoline; and soluble in acetone, alcohol, benzol, carbon disulfide and chloroform. Other types of accelerators include NOBS Special described as N-oxydiethylene benzothiazole-2-sulfenamide, and available from American Cyanamid Company; and Santocure NS described as N-tert-butyl-2-benzothiazole sulfenamide, and available from Monsanto Chemical Company. These two accelerators are described in Rubber Red Book, 10th edition, 1955-56, published by Rubber Age, New York, New York.

It is to be understood that each of the various types of compounding ingredients may be used singly or mixtures of various ingredients performing a certain function may be employed. It is sometimes preferred, for example to use mixtures of plasticizers rather than a single material.

The various ingredients in the propellant composition may be mixed on a roll mill or an internal mixer such as a Banbury or a Baker-Perkins dispersion blade mixer may be employed. The binder forms a continuous phase in the propellant with the oxidant as the discontinuous phase.

Rocket grains are formed by compression molding, injection molding, injecting molding, or extrusion.

The curing temperature will be limited by the oxidizer employed in some cases but will generally be in the range between 70 and 250° F., preferably between 70 and 200° F.

The curing time must be long enough to give required creep resistance and other mechanical properties in the propellant. The time will generally range from around three hours when the higher curing temperatures are employed to seven days when curing is effected at lower temperatures.

While this invention has been described using as the binder for propellant compositions a copolymer of a conjugated diene with a polymerizable heterocyclic nitrogen base of the pyridine series, such as vinylpyridine and various alkyl-substituted derivatives, it is to be understood that the corresponding quinoline and isoquinoline compounds are also applicable, i.e., vinylquinolines, vinylisoquinolines and various alkyl-substituted derivatives of these compounds.

#### Example I

Two solid propellants were prepared having compositions as follows:

|                                             | Parts by weight |    |
|---------------------------------------------|-----------------|----|
|                                             | 1               | 2  |
| Oxidizer (NH <sub>4</sub> NO <sub>3</sub> ) | 85              | 85 |
| Binder                                      | 15              | 15 |
| Miori blue                                  | 2               | 2  |
| Magnesium oxide                             | 1               | 0  |

The binder composition was prepared using a 90/10 butadiene/2-methyl-5-vinylpyridine copolymer having a Mooney value (ML-4) of 20. The binder composition was prepared in accordance with the following formulation:

|                                                   | Parts by weight |
|---------------------------------------------------|-----------------|
| Butadiene/2-methyl-5-vinylpyridine copolymer      | 100             |
| Carbon black, med. abrasion furnace               | 20              |
| Benzophenone                                      | 20              |
| N,N-dimethyl-S-tert-butylsulfenyl dithiocarbamate | 1               |
| Sulfur                                            | 0.75            |
| Zinc oxide                                        | 3               |
| Aerosol OT <sup>1</sup>                           | 1               |
| Flexamine <sup>2</sup>                            | 3               |

<sup>1</sup> Dioctyl ester of sodium sulfosuccinic acid.

<sup>2</sup> Physical mixture containing 25 percent of a complex diarylamine-ketone reaction product and 35 percent of N,N'-di-phenyl-p-phenylenediamine.

The various ingredients making up the propellants were mixed in a Baker-Perkins dispersion blade mixer until a substantially homogeneous mixture was obtained with the binder forming the continuous phase in the final composition. Material from each composition was extruded into a sheet 0.25 inch in thickness from which tensile specimens were stamped out prior to curing. Burning rate strands were extruded. Propellant grains were also prepared from each of the compositions. All specimens were cured 24 hours at 170° F. Mechanical properties and ballistic data were determined on both fresh and aged compositions. Results were as follows:

|                                                     | 1 | 2 |
|-----------------------------------------------------|---|---|
| Fresh propellant:                                   |   |   |
| Ballistic data:                                     |   |   |
| Strand data:                                        |   |   |
| r at 1,000 p.s.i., in./sec. <sup>1</sup> -----      |   |   |
| n, pressure exponent <sup>2</sup> -----             |   |   |
| Motor data:                                         |   |   |
| r at 1,000 p.s.i., in./sec. <sup>1</sup> -----      |   |   |
| n, pressure exponent <sup>2</sup> -----             |   |   |
| c*, ft./sec. (characteristic exhaust velocity)----- |   |   |
| Smoke <sup>4</sup> -----                            |   |   |
| Mechanical properties:                              |   |   |
| Ultimate stress (tensile), p.s.i.-----              |   |   |
| Ultimate elongation, percent-----                   |   |   |
| Modulus of elasticity, p.s.i.-----                  |   |   |
| Propellant aged 2 weeks at 170° F.:                 |   |   |
| Ballistic data—Strand data:                         |   |   |
| r at 1,000 p.s.i., in./sec. <sup>1</sup> -----      |   |   |
| n, pressure exponent <sup>2</sup> -----             |   |   |
| Mechanical properties:                              |   |   |
| Ultimate stress (tensile), p.s.i.-----              |   |   |
| Ultimate elongation, percent-----                   |   |   |
| Modulus of elasticity, p.s.i.-----                  |   |   |
| Propellant aged 1 month at 170° F.:                 |   |   |
| Ballistic data—Strand data:                         |   |   |
| r at 1,000 p.s.i., in./sec. <sup>1</sup> -----      |   |   |
| n, pressure exponent <sup>2</sup> -----             |   |   |
| Mechanical properties:                              |   |   |
| Ultimate stress (tensile), p.s.i.-----              |   |   |
| Ultimate elongation, percent-----                   |   |   |
| Modulus of elasticity, p.s.i.-----                  |   |   |

<sup>1</sup> Burning rate.

<sup>2</sup> Pressure exponent in  $r = aP_0^n$  where  $a$  is a constant and  $P_0$  is average chamber pressure.

<sup>3</sup> Average values from a series of 22 firings on grains from a series of batches all prepared in the same manner.

<sup>4</sup> Percent attenuation of light beam in path of exhaust.

These data show that when using magnesium oxide tensile strength and elongation values remain high upon aging and that the modulus of elasticity is affected only slightly. The burning rate of the propellant is only slightly altered and a substantial decrease in smoke evolution is obtained by the addition of magnesium oxide.

#### Example II

Propellants were prepared having the following compositions in parts by weight.

| Run No.                                     | 1   | 2    | 3    | 4   | 5    |
|---------------------------------------------|-----|------|------|-----|------|
| Oxidizer (NH <sub>4</sub> NO <sub>3</sub> ) | 85  | 82.5 | 82.5 | 85  | 82.5 |
| Binder                                      | 15  | 17.5 | 17.5 | 15  | 17.5 |
| Miori blue                                  | 2   | 2    | 2    | 2   | 2    |
| MgO                                         |     |      | 0.8  | 1.0 | 0.5  |
| ZnO                                         | 0.3 | 0.8  |      | 0.3 | 0.3  |

The binder employed in runs 1 to 5 above was prepared according to the following formulation.

|                                                   | Parts by weight |
|---------------------------------------------------|-----------------|
| Butadiene/2-methyl-5-vinylpyridine copolymer      | 100             |
| Carbon black, medium abrasion furnace             | 20              |
| Benzophenone                                      | 20              |
| N,N-dimethyl-S-tert-butylsulfenyl dithiocarbamate | 1               |
| Sulfur                                            | 0.75            |
| Aerosol OT                                        | 1               |
| Flexamine                                         | 3.0             |

The ingredients were mixed and specimens prepared as in Example I. All specimens were cured 24 hours at

170° F. Physical properties and ballistic data of the fresh and aged compositions are tabulated below.

from the group consisting of ammonium dichromate, potassium dichromate, iron oxide, a complex cyanide of

| Run No.                             | 1<br>439-B-53 | 2<br>628-A-1 | 3<br>627-A-1 | 4<br>493-A-1 | 5<br>492-A-1 |
|-------------------------------------|---------------|--------------|--------------|--------------|--------------|
| Fresh propellant:                   |               |              |              |              |              |
| Strand burning data:                |               |              |              |              |              |
| r at 1,000 p.s.i. (in./sec.)        | 0.161         | 0.152        | 0.155        | 0.154        | 0.153        |
| n, pressure exponent                | 0.51          | 0.50         | 0.49         | 0.53         | 0.55         |
| Mechanical properties:              |               |              |              |              |              |
| Ultimate stress (p.s.i.)            | 211           | 274          | 219          | 184          | 187          |
| Ultimate elongation (percent)       | 25.6          | 17.2         | 24.1         | 23.9         | 25.1         |
| Modulus elasticity (p.s.i.)         | 2,300         | 3,038        | 1,890        | 1,800        | 2,200        |
| Propellant aged 1 week at 170° F.:  |               |              |              |              |              |
| Strand burning data:                |               |              |              |              |              |
| r at 1,000 p.s.i. (in./sec.)        | 0.157         |              |              | 0.160        | 0.151        |
| n, pressure exponent                | 0.51          |              |              | 0.58         | 0.54         |
| Mechanical properties:              |               |              |              |              |              |
| Ultimate stress (p.s.i.)            | 205           |              |              | 274          | 245          |
| Ultimate elongation (percent)       | 20.9          |              |              | 18.0         | 22.8         |
| Modulus elasticity (p.s.i.)         | 1,800         |              |              | 2,100        | 1,400        |
| Propellant aged 2 weeks at 170° F.: |               |              |              |              |              |
| Strand burning data:                |               |              |              |              |              |
| r at 1,000 p.s.i. (in./sec.)        | 0.157         | 0.151        | 0.151        | 0.161        | 0.153        |
| n, pressure exponent                | 0.50          | 0.52         | 0.46         | 0.51         | 0.54         |
| Mechanical properties:              |               |              |              |              |              |
| Ultimate stress (p.s.i.)            | 194           | 279          | 178          | 296          | 295          |
| Ultimate elongation (percent)       | 14.7          | 10.8         | 13.4         | 16.0         | 19.7         |
| Modulus elasticity (p.s.i.)         | 2,000         | 3,108        | 1,778        | 2,400        | 2,000        |
| Propellant aged 4 weeks at 170° F.: |               |              |              |              |              |
| Strand burning data:                |               |              |              |              |              |
| r at 1,000 p.s.i. (in./sec.)        |               | 0.155        | 0.152        | 0.162        | 0.152        |
| n, pressure exponent                |               | 0.55         | 0.51         | 0.53         | 0.55         |
| Mechanical properties:              |               |              |              |              |              |
| Ultimate stress (p.s.i.)            | 175           | 250          | 126          | 309          | 291          |
| Ultimate elongation (percent)       | 12.1          | 9.2          | 14.0         | 13.4         | 17.3         |
| Modulus elasticity (p.s.i.)         | 2,100         | 3,415        | 1,398        | 2,900        | 2,100        |

The data reported in Example II further demonstrate the improved aging characteristics resulting from the addition of a minor amount of magnesium oxide to a propellant composition. These data also indicate that both magnesium oxide and zinc oxide are necessary to obtain the improved aging characteristics. The binder of Example I contained zinc oxide in the recipe so that both zinc oxide and magnesium oxide were present in the propellant formulation identified as run 1 of Example I.

Variations and modifications are possible within the scope of the disclosure of the present invention, the essence of which is the discovery that the addition of a minor amount of magnesium oxide to a solid rocket fuel containing a conjugated diene-heterocyclic nitrogen base copolymer binder results in surprising improvements in aging characteristics of the rocket fuel and also results in marked reduction by smoke evolution.

That which is claimed is:

1. A solid propellant composition consisting essentially of from 50 to 90 parts by weight of a solid inorganic oxidizing salt and 10 to 50 parts by weight of a sulfur-cured binder consisting essentially of a copolymer of a conjugated diene containing 4 to 6 carbon atoms per molecule and at least one



substituted heterocyclic nitrogen base selected from the group consisting of pyridine, quinoline, an alkyl substituted pyridine and an alkyl substituted quinoline, wherein the total number of carbon atoms in the nuclear alkyl substituents is not more than 15 and wherein R is selected from the group consisting of hydrogen and a methyl radical, 0 to about 50 parts by weight per 100 parts of copolymer of carbon black, 0 to about 100 parts by weight per 100 parts of copolymer of a rubber plasticizer, 0 to about 10 parts by weight per 100 parts of copolymer of a wetting agent, 0 to about 3 parts by weight per 100 parts of copolymer of an antioxidant, 0 to about 5 parts by weight per 100 parts of copolymer of a vulcanization accelerator, and 0 to about 5 parts by weight per 100 parts of copolymer of zinc oxide; 0 to about 15 parts by weight per 100 parts of oxidizing salt and binder mixture of a burning rate catalyst selected

nickel, a complex cyanide of copper, and a complex cyanide of iron; and about 0.2 to about 5 parts by weight per 100 parts of oxidizing salt and binder mixture of magnesium oxide.

2. The composition of claim 1 wherein the oxidizing salt is ammonium nitrate.

3. The composition of claim 3 wherein the oxidizing salt is ammonium perchlorate.

4. The composition of claim 1 wherein the oxidizing salt is potassium nitrate.

5. The composition of claim 1 wherein the oxidizing salt is potassium perchlorate.

6. The composition of claim 1 wherein the copolymer is prepared from a mixture of monomers comprising 1,3-butadiene and 2-methyl-5-vinylpyridine.

7. The composition of claim 1 wherein the copolymer is prepared from a mixture of monomers comprising isoprene and 2-vinylpyridine.

8. The composition of claim 1 wherein the copolymer is prepared from a mixture of monomers comprising styrene and 4-vinylpyridine.

9. The composition of claim 1 wherein the burning rate catalyst is a complex cyanide of iron.

10. The composition of claim 1 wherein the burning rate catalyst is miliori blue.

11. The composition of claim 1 wherein the burning rate catalyst is ammonium dichromate.

12. The composition of claim 1 wherein the burning rate catalyst is potassium dichromate.

13. The composition of claim 1 wherein the burning rate catalyst is iron oxide.

14. In the manufacture of a solid propellant composition consisting essentially of from about 50 to about 90 parts by weight of a solid inorganic oxidizing salt, about 10 to about 50 parts by weight of a zinc oxide-containing, sulfur-cured binder comprising a copolymer of a conjugated diene containing 4 to 6 carbon atoms per molecule and at least one



substituted heterocyclic nitrogen base selected from the group consisting of pyridine, quinoline, an alkyl substituted pyridine and an alkyl substituted quinoline, wherein

the total number of carbon atoms in the nuclear alkyl substituents is not more than 15 and wherein R is selected from the group consisting of hydrogen and a methyl radical and 0 to about 15 parts by weight per 100 parts of oxidizing salt and binder mixture of a burning rate catalyst selected from the group consisting of ammonium dichromate, potassium dichromate, iron oxide, a complex cyanide of nickel, a complex cyanide of copper, and a complex cyanide of iron, wherein the ingredients are in-

corporated and cured, the improvement comprising admixing about 0.2 to about 5 parts by weight per 100 parts of oxidizing salt and binder mixture of magnesium oxide with the ingredients of the propellant composition during the step of incorporation; and curing the magnesium oxide-containing mixture at about 70 to about 250° F. for about 3 hours to about 7 days.

No references cited.

UNITED STATES PATENT OFFICE  
CERTIFICATE OF CORRECTION

Patent No. 3,010,814

November 28, 1961

Donald E. Carr

It is hereby certified that error appears in the above numbered patent requiring correction and that the said Letters Patent should read as corrected below.

Column 8, line 38, for the claim reference numeral "3" read -- 1 --.

Signed and sealed this 3rd day of July 1962.

(SEAL)

Attest:

ERNEST W. SWIDER  
Attesting Officer

DAVID L. LADD  
Commissioner of Patents